

## UNITED STATES PATENT OFFICE.

CHARLES CUMINGS, OF CHICAGO, ILLINOIS, ASSIGNOR TO COMMERCIAL STEEL COMPANY, A CORPORATION OF ILLINOIS.

## MANUFACTURE OF STEEL.

No Drawing. Continuation of application Serial No. 282,579, filed March 12, 1919. This application filed December 23, 1919. Serial No. 347,004.

To all whom it may concern:

Be it known that I, CHARLES CUMINGS, a subject of Great Britain, and resident of Chicago, county of Cook, and State of Illinois, have invented certain new and useful Improvements in the Manufacture of Steel, of which the following is a specification.

This application is filed as a continuation of and a substitute for an application for patent filed by myself March 12, 1919, Serial No. 282,579 for process and method of manufacturing steel.

The invention relates to the manufacture of steel and contemplates a treatment of the molten bath, preferably employed immediately prior to pouring, which has been found to secure in the completed product marked improved physical properties as compared with steels of like or similar chemical composition heretofore produced. The invention is believed to be applicable to the production of steel and so-called steel alloys of any usual chemical analysis, and in the practice of the invention no substantial change in the chemical analysis of the product has been found to result from the use of the novel step or steps of the improved process and no such change is now believed to occur, at least so far as the quantities of the ingredients usually determined in the analysis of steels or now known to exist in steel, are concerned.

The object of the invention is the provision of the improved method of manufacturing steel hereinafter described and claimed and the improved product resulting therefrom.

The invention may be practiced when the molten bath has been prepared in the ordinary manner and the desired carbon or carbon and alloy content of the finished product secured in the usual manner and the steel is otherwise considered ready to pour into the ladle or ingot mold. When the bath has reached this condition, if the method of treatment specifically described is to be used, it is desirable to add to the metal bath a quantity of ore such as tungsten concentrates or chrome ore, or a mixture of these ores. A desirable mixture of materials for this purpose may consist of equal parts of tungsten concentrates containing about 45% of tungstic acid and

chrome ore containing about 45% of chrome oxide. A suitable amount of this mixture is found to be 40 pounds to the ton of metal. Other metallic ores having like qualities may be substituted for or mixed with those named.

After the addition of the ores as described the bath is preferably poled and the ebullition is allowed to subside. In the preparation of a bath of from one to five tons in an open hearth or electric furnace this will take place in about fifteen minutes.

The method of treatment which is at present preferred, and for which the above step of adding ores is a preparation, is the addition to the bath of an explosive mixture and allowing the mixture to become ignited on or beneath the surface of the molten metal. The explosive mixture may and preferably does comprise an intimate mixture of fuel, either solid, liquid or gaseous, with oxidizing material in solid or liquid form. The oxidizing agent may be a single material or a combination of materials mixed together. An explosive mixture which is found to give satisfactory results is composed of two to four pounds of finely pulverized charcoal, about four ounces of powdered potassium chlorate, and about eight ounces of barium dioxide. The quantity of the materials named is sufficient for one ton of molten metal.

After the introduction of the explosive mixture the bath is allowed to stand for about five minutes, in the case of a bath of from one to five tons, to allow the action to subside, when it may be poured into the ladle or mold. Larger baths than those mentioned will require larger quantities of materials, and it may be desirable to allow longer periods of time for subsidence of action.

It is exceedingly difficult to ascertain exactly what occurs in the bath when the materials named are added thereto. The most satisfactory theory yet arrived at in explanation of the results attained is believed to be as follows:

The ores are useful only as protective agents to prevent oxidation of the carbon content of the metal and of the metal itself under the sudden and considerable rise in temperature resulting from the combustion of the explosive mixture. This theorv

60

70

75

80

85

90

95

105

derives support from the fact that chemical analysis of the completed product shows none, or but a trace of the tungsten or chromium in carbon steel, as distinguished 5 from alloy steel, the amount being in no case sufficient, as is now believed, to affect materially the physical characteristics and thus account for the improvement in physical properties secured in the product by the 10 use of the invention.

The utilization of the explosive mixture is at present regarded as a practicable and effective method of producing a violent agitation accompanied by a sudden shock and by 15 a substantial rise in temperature. This action differs in kind from such action as is obtained by poling or blowing, or by the introduction of either fuel alone or oxidizing agents alone or even by the introduction of 20 mixed fuel and oxidizing agents gradually. In all of these cases the bath is affected gradually. Even the generation of gases in contact with the bath in all cases of which I am aware previous to my invention has 25 been a gradual action since the gas was only generated as successive molecules came into contact with the bath.

The substantial rise in temperature produced in the bath by the combustion of the 30 explosive mixture is believed to be of importance as rendering the bath more fluid and mobile. Whether the gases produced by the combustion of the explosive mixture so react with the gasses occluded in the molten 35 metal as to modify the results has not yet been determined. It is suggested, however, that the large quantity of gas thus generated or released at the surface of or within the bath serves to sweep out occluded 40 gases and particles of slag which would otherwise remain and that the amount of occluded gas and slag contained in the finished product is thus reduced. The higher 45 temperature of the bath may also reduce the solubility of both gaseous and solid or molten materials in the metal and the elimination 50 of these substances is, of course, assisted by the greater fluidity of the bath. Furthermore, it is known that the bubbling 55 of gases through liquids containing finely divided matter in suspension frequently promotes elimination of the suspended matter, and it is suggested that the bubbling of the gaseous products of the combustion of the explosive 60 mixture may have this effect with reference to suspended slag and occluded gases contained in the bath.

In any event the results obtained are at 65 present believed to be due in part to a more complete elimination of impurities, in part to a thorough diffusion of the remaining impurities, of any, throughout the mass, thus making the product denser and more perfectly homogeneous, and in part to the 65 production of a finer grain in the product.

Whatever the explanation of the operation of the invention, tests of the completed product, as compared with steel of substantially the same chemical analysis made by processes heretofore known and subjected to 70 the same heat treatment, if any, have shown an increase of tensile strength of from 50% upward, and corresponding improvement in other physical properties, as a result of the application of the invention. Photo-micrographs of steel which has been produced by the process above described show a more perfectly regular reticulation than that produced by processes heretofore known, and in the samples so far tested by photo-micrographs no trace of impurity splotches has 75 been detected.

Applicant disclaims the treatment of metal by the mechanical or chemical effect or combination thereof, which may be produced by the ignition of a mixture of granulated metallic aluminum and metallic oxides in or on a bath of molten metal or the ignition of such a mixture containing scavenging materials such as alloys of some or all 80 of silicon, manganese, aluminum, titanium or magnesium. The charge, such as mentioned, does not produce a sufficiently sudden effect to bring about the improvement which applicant has discovered that the 85 shock which may be produced by an explosion does bring about.

While the treatment embodying the invention has been described as carried out when the bath has been prepared in its desired chemical analysis, it may in some cases be found desirable to apply it at other stages of the manufacture and later to add some of the constituents desired to have present in the finished product. This and many 105 other modifications may be made in the carrying out of the process without departing from the spirit of the invention.

I claim as my invention:

1. The process of preparing metal which 110 comprises subjecting a molten bath of the metal to an agitation in the nature of a sudden shock of sufficient intensity to produce a substantial improvement in the tensile strength and other physical properties of the 115 finished product.

2. The process of preparing metal which 120 comprises subjecting a molten bath of the metal to a sudden shock accompanied and followed by violent agitation said shock being of sufficient intensity whereby in combination with said agitation to produce a substantial improvement in the tensile strength and other physical properties of the finished product.

3. The process of preparing metal which 125 comprises subjecting a molten bath of the metal to a sudden shock striking widely and substantially instantaneously through the mass of the bath followed immediately by 130

- a violent agitation in the nature of flow of the metal said shock being of sufficient intensity whereby in combination with said agitation to produce a substantial improvement in the tensile strength and other physical properties of the finished product.
4. The process of preparing metal which comprises subjecting a molten bath of the metal to an agitation in the nature of a sudden shock, of sufficient intensity to produce a substantial improvement in the tensile strength and other physical properties of the finished product, said shock accompanied by substantial rise of temperature.
5. The process of preparing metal which comprises subjecting a molten bath of the metal to a sudden shock of sufficient intensity to produce a substantial improvement in the tensile strength and other physical properties of the finished product, said shock accompanied and followed by violent agitation and substantial rise of temperature.
6. The process of making steel which comprises subjecting a molten ferrous bath to an agitation in the nature of a sudden shock of sufficient intensity to produce a substantial improvement in the tensile strength and other physical properties of the finished product.
7. The process of making steel which comprises subjecting a molten ferrous bath to an agitation in the nature of a sudden shock of sufficient intensity to produce a substantial improvement in the tensile strength and other physical properties of the finished product, said shock accompanied by a violent agitation.
8. The process of making steel which comprises subjecting a molten ferrous bath to a sudden shock of sufficient intensity to produce a substantial improvement in the tensile strength and other physical properties of the finished product, said shock accompanied and followed by a violent agitation and substantial rise in temperature.
9. The process of making steel which comprises preparing a bath of metal of substantially the composition desired in the finished product and subjecting the bath to an agitation in the nature of a sudden shock.
10. In the preparation of steel the process which comprises preparing a bath of molten metal and adding to said bath a single integral mass of material of such a nature and in such a quantity as to generate large volumes of gas substantially instantaneously whereby to subject the bath to a sudden shock of sufficient intensity to produce a substantial improvement in the tensile strength and other physical properties of the finished product.
11. The process of making steel which comprises preparing a bath of molten metal of substantially the analysis desired in the finished product, and adding to said bath a single integral mass of material in such quantity and of such a nature to generate large quantities of gas substantially instantaneously.
12. The process of making steel which comprises preparing a bath of molten metal of substantially the analysis desired in the finished product, adding to said bath a quantity of non-ferrous ore, allowing ebullition to subside, and subjecting the bath to the action of an agitation in the nature of a sudden shock accompanied and followed by a substantial rise in temperature.
13. The process of making steel which comprises preparing a molten ferrous bath and adding to said bath a single integral mass of an intimate mixture of fuel and an oxidizing agent in such a quantity as to substantially instantaneously generate large volumes of gas.
14. The process of making steel which comprises preparing a molten ferrous bath and adding to said bath a single integral mass of an intimate mixture of finely divided fuel in solid form and an oxidizing agent in such a quantity as to substantially instantaneously generate large volumes of gas.
15. The process of making steel which comprises adding to a molten ferrous bath of metal of substantially the analysis desired in the finished product a single integral mass of an intimate mixture of fuel and an oxidizing agent in such a quantity as to substantially instantaneously generate large volumes of gas.
16. The process of making steel which comprises adding to a molten bath of metal, of substantially the analysis desired in the finished product, a quantity of non-ferrous ore, allowing ebullition to subside and thereafter adding a quantity of an intimate mixture of a fuel and an oxidizing agent.
17. The process of making steel which comprises adding to a molten bath of metal, of substantially the analysis desired in the finished product, a quantity of material adapted to prevent substantial change of carbon content during subsequent treatment, and adding to the bath a quantity of an intimate mixture of fuel and an oxidizing agent.
18. The process of making steel which comprises adding to a bath of molten metal, of substantially the analysis desired in the finished product, a quantity of tungsten concentrates, poling the mass, allowing the ebullition to subside, and adding to the bath a quantity of an intimate mixture of fuel and an oxidizing agent.
19. The process of making steel which comprises adding to a bath of molten metal, of substantially the analysis desired in the finished product, a quantity of a mixture of equal parts of tungsten and chrome.

mium ores, poling the mass, allowing the ebullition to subside, and adding to the bath a quantity of an intimate mixture of fuel and an oxidizing agent.

- 5 20. The process of making steel which comprises adding to a bath of molten metal, of substantially the analysis desired in the finished product, a quantity of material adapted to prevent substantial change in 10 carbon content of the bath during subsequent treatment, and adding a quantity of an intimate mixture of finely divided fuel and potassium chlorate.

- 15 21. The process of making steel which comprises adding to a bath of molten metal, of substantially the analysis desired in the finished product, a quantity of material adapted to prevent substantial change in carbon content of the bath during subsequent 20 treatment, and adding a quantity of an intimate mixture of finely divided fuel, potassium chlorate and barium dioxide.

- 25 22. The process of making steel which comprises adding to a bath of molten metal, of substantially the analysis desired in the finished product, a quantity of material adapted to prevent substantial change in carbon content of the bath during subsequent 30 treatment, and thereafter adding a quantity of an intimate mixture of finely divided fuel in solid form and potassium chlorate.

- 35 23. The process of making steel which comprises adding to a molten bath of metal of substantially the composition desired in the finished product a quantity of material adapted to prevent substantial change in composition during subsequent treatment, adding to the thus treated bath an intimate 40 mixture of finely divided carbon and potassium chlorate.

- 45 24. Process of refining molten metal consisting in adding an explosive agent acting to mechanically expel gases and impurities whereby to substantially improve the tensile strength and other physical properties of the finished product.

- 50 25. Process of treating molten metal consisting in adding a scavenging charge and an explosive agent acting to mechanically expel gases and impurities whereby to substantially improve the tensile strength and other physical properties of the finished product.

- 55 26. The process of making steel which comprises preparing a molten bath of the steel of substantially the carbon content de-

sired in the finished product, adding an explosive agent in such a quantity as to produce a shock in the metal of sufficient intensity to provide a substantial improvement in the tensile strength and other physical properties of the finished product without effecting the carbon content of the bath, and then pouring the metal after completion of the explosive reaction.

60 27. The process of making steel which comprises preparing a molten bath of the metal having a carbon content desired for the finished product, adding to the bath 70 material to prevent a reduction of the carbon content by the subsequent treatment, adding an explosive agent to the bath to produce a shock therein of sufficient intensity to improve the tensile strength and 75 other physical properties of the finished product without effecting the desired analysis, and then pouring the metal after completion of the explosive reaction.

80 28. The process of making steel which comprises preparing a molten bath of metal, holding the bath in such a manner that it may yield freely to pressure and subjecting the bath to a shock of explosive violence of sufficient intensity to produce substantial 85 improvement in the tensile strength and other physical properties of the finished product.

85 29. The process of making steel which comprises preparing a molten bath of metal 90 having the carbon content desired in the finished product, adding a charge of scavenging material to the bath, allowing ebullition to subside, holding the bath in such a manner as to be free to yield to pressure and subjecting the bath to a shock of explosive violence of sufficient intensity to produce substantial improvement in the tensile strength and other physical properties of the finished product.

100 30. The process of making steel which comprises preparing a molten bath of metal having the carbon content desired in the finished product, adding a charge of non-ferrous ore, allowing the ebullition to subside and drawing the slag from the surface, holding the bath in such a manner as to be free to yield to pressure and subjecting the bath to a shock of explosive violence of sufficient intensity to produce substantial 105 improvement in the tensile strength and other physical properties of the finished product.

CHARLES CUMINGS.